

## UNITED STATES PATENT OFFICE

2,126,936

## TEXTILE FINISHING MATERIAL

Eugene Welgamuth Wall, Philadelphia, Pa., assignor to Kali Manufacturing Company, Philadelphia, Pa., a corporation of Pennsylvania

No Drawing. Application March 23, 1936,  
Serial No. 70,553

## 2 Claims. (Cl. 134—11)

This invention relates to textiles, and is concerned primarily with the application of a material to fabrics to impart crease-proofing or crush-proofing properties, as well as a permanent finish thereto.

At the present time it is a known expedient in the textile arts to avail of certain synthetic resins, as a finishing agent of this type. However, the use of such synthetic resins requires a fairly high temperature for drying and calendering of the fabric.

With the foregoing in mind, this invention has in view, as its foremost objective, the provision of a finishing agent of the type above referred to, which is intended for use in conjunction with textiles to provide for the drying and calendering of the fabric at a lower temperature than has heretofore been necessary.

More particularly, this invention has in view, as an objective, the provision of a finishing agent of the type above noted, which is identified as including a sucrose acetate as its characteristic element.

This invention proposes the use of sucrose octa-acetate which is now available to the buying public as such.

A further object of this invention is to provide a solution which includes sucrose octa-acetate, and which solution is readily adaptable for application to textile materials for the usual proofing or finishing purposes.

In carrying out this thought in a practical embodiment, the sucrose octa-acetate is dissolved in a solvent which may be any one of a wide range of materials, as will be pointed out in detail hereinafter. This solution is applied to the textile materials in the conventional manner, whereupon subsequent drying and calendering operations impart a permanent finish to the fabrics.

Yet another object of the present invention is to provide a finishing solution of the character above noted, which also includes a softening or modifying agent.

Various other more detailed objects and advantages will in part become apparent, and in part be hereinafter stated, as the description of the invention proceeds.

The invention, therefore, comprises a finishing material intended for use with textiles, which is identified by the presence of sucrose octa-acetate, which is put in solution in an appropriate solvent, and which solution also contains a softening agent.

The present invention proposes the finishing

of various types of fabrics, which may be in the form of piece goods, such as woven or knitted piece goods that may be made from cotton, linen, silk, rayon or other artificial cellulose fibres, wool, jute, hemp, ramie, or any fabrics made up of compositions of these materials.

The invention also proposes the application of the finishing material to the yarn prior to weaving or knitting into the ultimate fabric. When the material is used as a finishing agent, it is particularly adapted to impart a permanent finish or stiffening effect to such goods, as collar fabrics, coat canvas, and other similar fabrics where stiffness is a desired property.

In preparing the finishing material contemplated by this invention, sucrose octa-acetate, together with a softening agent, which may be of any one of the following: vegetable oils such as castor, olive, linseed; animal oils such as neat's-foot; fatty acids such as oleic, stearic; paraffine; spermaceti; higher alcohols, as for example, cetyl, lauryl, oleyl; petroleum derivatives, such as petrolatum and various petroleum oils; sulphonated oils and fats, such as sulphonated castor oil, sulphonated olive oil, sulphonated tallow and similar derivatives; sulphonated higher alcohols, such as Gardinol, Aviroil and similar products or substituted sulphonated naphthalenes such as Nekal, is put in solution with a solvent which may be any one of the following listed materials: methyl alcohol, ethyl alcohol, ethyl acetate and other esters of this series; acetone, carbon tetrachloride, ethylene dichloride, trichlorethylene, petroleum spirits, turpentine, pine oil, turpene, benzol and its homologues. Under certain conditions it may be desirable to use a modifying agent for the sucrose octa-acetate, and this agent may be shellac, sandarac, damar, rosin, cummar, or a wax such as beeswax or Japan wax.

The sucrose octa-acetate is present in the ultimate solution in a proportion ranging from 1 to 5% of the ultimate product, and the softening agent is also present in a proportion within the same range. The solution of this invention will include the sucrose octa-acetate and softening agent in their combined form up to 5% of the whole. For instance, the solution may contain about 2% of sucrose octa-acetate and 1% of the softening agent, the two together making up 3% of the entire solution.

After the finishing solution has been applied to the fabric, either before or after weaving, the latter is subjected to the usual drying and calendering operations, which may be carried out at

temperatures appreciably lower than has heretofore been necessary under similar conditions involving the application of a finishing or proofing agent.

5 A particular advantage of the present finishing and proofing agent is that it is entirely unaffected by any washing of the fabric to which this material may be applied.

10 While preferred specific embodiments of the invention are hereinbefore set forth in detail, it is to be understood that I am not to be limited to the exact compositions above enumerated because various modifications of these details may be provided in putting the invention into practice, within the purview of the appended claims.

15 I claim:—

1. A dilute liquid textile finishing material of the character described, consisting of a solution which consists of a solvent for sucrose acetate and a sucrose acetate together with a softening agent for sucrose octa-acetate, the sucrose acetate and softening agent each being present in proportions ranging from 1 to 5% of the solution. 5

2. A dilute liquid textile finishing material of the character described, consisting of a solvent for sucrose octa-acetate, and sucrose octa-acetate, together with a softening agent for sucrose octa-acetate, said sucrose octa-acetate and softening agent being present in equal amounts and in a proportion ranging from 2% to 5% of the entire solution. 10 15

EUGENE WOLGAMUTH WALL.